

## UNITED STATES PATENT OFFICE.

HENRY R. POWER, OF NIAGARA FALLS, NEW YORK, ASSIGNOR TO THE CARBORUNDUM COMPANY, OF NIAGARA FALLS, NEW YORK, A CORPORATION OF PENNSYLVANIA.

## ABRASIVE COMPOSITION.

No Drawing.

Application filed April 5, 1921. Serial No. 458,803.

To all whom it may concern:

Be it known that I, HENRY R. POWER, a citizen of the United States, residing at Niagara Falls, in the county of Niagara and State of New York, have invented a new and useful Improvement in Abrasive Compositions, of which the following is a full, clear, and exact description.

The abrasive or grinding composition herein referred to is for grinding metal surfaces, such as valve seats for motor engines or for any grinding operation where it is proposed to make a tight joint between two metal surfaces.

The abrasive composition I have produced is a paste made up of particles of abrasive material, water and one of that peculiar class of colloidal bodies called gums. I here refer to the true gums and use the term "gum" in its strictly chemical sense. Gums are either soluble in cold water, giving a heavy, thick liquid, or they simply swell up in cold water. Either type of gum in water may be made into a jelly by the use of basic lead acetate and other chemicals, such a jelly being satisfactory to form a paste with abrasive particles. Among the chemicals that may be used with solutions of gum as thickeners to form a jelly are borax, ammonium oxalate, mercuric chloride, iron salts, potassium and sodium silicate.

In particular, gums follow the type of gum arabic which is water soluble and gum tragacanth which simply swells up in water. I prefer to use gum tragacanth which I first form into a jelly by mixing with cold water in the proportion of four parts of gum to one hundred parts of water, though I may vary these proportions to get a heavier or lighter jelly when desired. The jelly thus prepared is thickened by a very slight quantity of chemical, preferably by the use of basic lead acetate. Then the abrasive particles are stirred into the jelly, giving a smooth paste of uniform consistency.

The advantages of this paste are that this is altogether a cold process, no heat being required at any stage. Moreover, gums are not capable of fermentation by yeast. Hence, no preservative is required to prevent the abrasive compound, made as herein stated, from molding.

The proportions of the abrasive composition I have found successful are

|                    |    |    |
|--------------------|----|----|
| Water              | 46 | 55 |
| Gum tragacanth     | 2  |    |
| Basic lead acetate | 1  |    |
| Glycerine          | 2  |    |
| Carborundum        | 50 | 60 |

Glycerine added to the paste has a tendency to prevent the evaporation of water and drying up of the paste.

I may vary any or all of the proportions of the formula as herein given, depending on the size of the abrasive particles, the strength of the paste required, etc. I may, moreover, use other than carborundum as the abrasive.

The water-mixed abrasive composition herein described has the advantage over grease grinding-pastes in the fact that grease is a lubricant and interferes with the cutting action of the abrasive particles, while the gum-jelly abrasive paste is not a lubricant and permits of a maximum amount of friction of the abrasive particles in the mixture.

I am aware that it has been proposed to make a scouring composition of powdered pumice, sand or the like mixed with silicate of soda and substances such as isinglass, gum tragacanth, starch or the like. Silicate of soda in such composition will tend to harden and is not satisfactory for the purposes for which my grinding composition is intended.

I claim:

1. An abrasive composition comprising abrasive particles and a gum, said composition being substantially free from either silicate of soda or oil, substantially as described.

2. An abrasive composition comprising abrasive particles, a gum and a thickener, said composition being substantially free from either silicate of soda or oil, substantially as described.

3. An abrasive composition comprising abrasive particles and a jelly made from a gum, said composition being substantially free from either silicate of soda or oil, substantially as described.

4. An abrasive composition comprising

abrasive particles, a jelly made from a gum and glycerine, said composition being substantially free from either silicate of soda or oil, substantially as described.

5 5. An abrasive composition comprising abrasive particles, gum tragacanth and basic lead acetate, substantially as described.

6. An abrasive composition comprising abrasive particles, gum, basic lead acetate and glycerine, substantially as described.

10 7. An abrasive composition consisting

principally of abrasive particles, a jelly made from a gum, a thickener and a hygroscopic substance, substantially as described.

8. An abrasive composition consisting <sup>15</sup> principally of abrasive particles, a jelly made from a gum, a thickener and glycerine, substantially as described.

In testimony whereof, I have hereunto set my hand.

HENRY R. POWER.